

Aug. 20, 1963

E. F. EMLEY

3,101,269

MAGNESIUM BASE ALLOYS

Filed Oct. 9, 1961



FIG. 1.



FIG. 2.



FIG. 4.

INVENTOR  
EDWARD FREDERICK EMLEY

BY  
Monon S. Nelson  
ATTY.

3,101,269

## MAGNESIUM BASE ALLOYS

Edward Frederick Emley, Manchester, England, assignor to Magnesium Elektron Limited, Manchester, England

Filed Oct. 9, 1961, Ser. No. 143,839

Claims priority, application Great Britain Oct. 18, 1960  
16 Claims. (Cl. 75—168)

This invention relates to magnesium zirconium alloys of the type disclosed in British Patent No. 511,137 and in particular to the binary alloy of magnesium and zirconium containing up to about 0.7% zirconium.

It is well known that magnesium alloys containing zirconium exhibit microstructures in which there are zirconium-rich cores in the centres of most of the grains. We have found that in the binary alloy these cores contain up to about 4% of zirconium in solution, although the maximum solubility of zirconium in the liquid alloy is only about 0.7% at normal casting temperatures. When such alloys are worked, the zirconium-rich cores become drawn out into zirconium-rich striations. These worked alloys show good resistance to loss of room temperature properties following annealing or hot working, and this phenomenon has been attributed to the effect of these zirconium-rich striations in restricting grain-growth.

Where such wrought alloys are to be used at high temperatures for long periods, for example in nuclear reactors, there is the possibility that the striations may gradually disappear owing to diffusion of zirconium throughout the microstructure with accompanying undesirable grain growth. There is further the possibility, for example in the case of the binary alloy, that the zirconium striations will become the seat of hydride precipitation arising through slow pick-up of hydrogen derived from moisture in the surrounding atmosphere. As a result of these effects, such alloys cannot be regarded as indefinitely stable for use at temperatures where these processes can occur.

In order to produce such worked alloys in the stable condition, it has been proposed to heat treat the worked alloys, for example extrusions of the binary alloy, at temperatures of about 600° C., in order to homogenise the alloy by diffusion of the zirconium. We have found this process to be very slow and accompanied by considerable grain growth, whilst the resultant alloys are still liable to precipitation of hydride. If such extrusions are deliberately heated in hydrogen, or a moist atmosphere, precipitation-free zones are formed near the grain boundaries, and the final product shows poor creep ductility at temperatures around 200–250° C.

In order to produce fine grained wrought zirconium alloys of high stability, we have subjected a cast or extruded billet to a precipitation treatment, so as to precipitate the zirconium as hydride (with possibly some nitride) by heat treatment in a suitable atmosphere containing available hydrogen, i.e. hydrogen, ammonia, moisture or other substance containing hydrogen in a form which can be taken up into the alloy. We have then extruded the billets and obtained fine grained alloys which are metallurgically stable at high temperatures because the zirconium can no longer diffuse or precipitate. These alloys are very resistant to grain growth at high temperature. Furthermore, since the grain boundaries after the working process no longer occupy the precipitation-free sites in the original billet, the alloys possess excellent creep ductility.

Table I illustrates the high ductility obtainable at 200° C. in accordance with the present invention when the hydriding step is carried out before rather than after extrusion. Thus extrusions C and D, which were hydrided

before extrusion, show elongations of 178 and 108% in comparison with extrusions E and F which were hydrided after extrusion and which show elongations of only 8 and 14%.

TABLE I

Creep Ductility Test Results at 200° C. of Binary Magnesium Zirconium Extruded Alloys

| Extrusion No. | Condition                          | Stress, t.s.i. | Time of Fracture (hrs.) | Elongation (percent) |
|---------------|------------------------------------|----------------|-------------------------|----------------------|
| 10            | Extruded only                      | 1.0            | 336                     | 58                   |
|               | do                                 | 1.5            | 50                      | 47                   |
| 15            | Hydrided and extruded              | 0.5            | 480                     | 178                  |
|               | do                                 | 1.0            | 43                      | 108                  |
|               | Homogenised, extruded and hydrided | 1.5            | 60                      | 8                    |
| 20            | do                                 | 2.0            | 9                       | 14                   |
|               | Homogenised, extruded              | 1.5            | 168                     | 50                   |
|               | Homogenised, hydrided, extruded    | 1.0            | 740                     | 42                   |
|               | do                                 | 1.5            | 48                      | 41                   |

Homogenisation treatment: 20 hrs. at 625° C. in boric acid. Hydriding treatment: 16 hrs. at 550° C. in moist hydrogen. Extrusion temperature: 400° C. approx.

The hydrogen treatment may be carried out at a temperature not less than 300° C., and preferably, not greater than 600° C., the time of treatment depending mainly on the maximum thickness of section of the billet or other workpiece. Thus at 550° C. in atmospheres such as dry hydrogen, wet hydrogen, wet CO<sub>2</sub>, or wet argon or steam, heat treatment times of the order of 6 hrs. per in. of section thickness are generally appropriate.

At lower temperatures, e.g. 400° C., the hydriding process occurs less readily, but satisfactory hydriding in reasonable times can be achieved if the components are first subjected to a shot-blasting treatment. This effect probably works in two ways: by contaminating the surface with iron, so providing electrolytic couples to assist decomposition of water vapour, and also by roughening the surface layers. As an alternative to shot-blasting, the surface may be roughened or activated in other ways, e.g. by treating it with salt solution or a solution containing an iron or other heavy metal salt. The lower hydriding temperatures produce finer precipitates than are obtained by hydriding at 550° C. and are consequently preferred where a stiffer product is desired.

The quantity of hydrogen which can readily be introduced into the alloy, e.g. at 550° C., is 200–250 cc. per g. of Zr content, and corresponds roughly with the formula ZrH<sub>2</sub>. We have found that under some circumstances, e.g. with shot-blasted specimens at 450° C. using steam or wet hydrogen, it is possible to introduce considerably higher proportions of hydrogen into the alloy, e.g. 400 cc. per g. of Zr content. The quantity of hydrogen should be at least 80 cc. per gram of zirconium. Also, the quantity of hydrogen in the alloy should be at least 0.002 percent by weight of the alloy, i.e. at least 22 cc. per 100 grams of the alloy. If desired, the hydrogen treatment may be carried out under pressure, e.g. at several atmospheres.

Other elements which may be included in the alloy are manganese up to 0.3% and rare earth metals up to 3% and thorium up to 3%, the rare earth metals and thorium together not exceeding 4%.

If desired, the rare earth metal can be pure cerium of low capture cross section for thermal neutrons, or a rare earth mixture containing at least 60% of neodymium. If rare earth metals or thorium are present, the hydrogen content of the final alloy will be correspondingly increased above the figures already indicated, since these elements will also be substantially precipitated as hydride. Exclusion of rare earth metals and thorium is,

Table I illustrates the high ductility obtainable at 200° C. in accordance with the present invention when the hydriding step is carried out before rather than after extrusion. Thus extrusions C and D, which were hydrided

however, desirable where the final alloy is to be welded, since their hydrides can decompose, giving rise to gas bubbles in the weld.

We have found that the concentration of zirconium in the cores in the middle of the grains is higher in the binary than in more complex alloys, and that hydride is not readily precipitated in the presence of some alloying elements, for example zinc. Zinc also lowers the solidus of the alloy, thus interfering with the process of homogenisation. Accordingly, it is preferred to use the binary alloy.

We have carried out welding tests on the binary magnesium zirconium alloys prepared in accordance with the present invention, and have found these alloys to show excellent weldability, the resulting welds being quite free from gas porosity.

According to one aspect of the present invention, therefore, a fine grained wrought magnesium alloy, which is metallurgically stable at high temperatures and possesses good creep ductility, has the following composition:

|      |                                                          |
|------|----------------------------------------------------------|
| Zr   | 0.1-1%.                                                  |
| H    | At least 0.002% (i.e. at least 22 cc. per 100 g. alloy), |
| Mn   | 0-0.3%.                                                  |
| R.E. | 0-3.0%.                                                  |
| Th   | 0-3.0%.                                                  |
| Mg   | The remainder.                                           |

the hydrogen content being at least 80 cc. per gram zirconium content, and the microstructure of the alloy being characterised by the absence of precipitation-free bands near the grain boundaries.

The maximum zirconium content preferred is 0.7% and the preferred hydrogen range is 22-350 cc. per 100 g. alloy, there being at least 100 cc. hydrogen per gram of zirconium content. The manganese contributes to the stiffness of the alloy at high temperatures, but adds to the capture cross section of the alloy for thermal neutrons. Accordingly, the manganese content is preferably restricted to not more than 0.2% and may usefully be 0.1-0.2% in cases where the presence of some manganese is desired. Since manganese and zirconium are to some extent incompatible in magnesium, the sum of the manganese and zirconium contents should not exceed 0.8% and the product of these contents expressed in percentage should not exceed 0.1.

A minimum zirconium content of 0.25% is also desirable, with a hydrogen content of 50-250 cc. per 100 g. alloy, but with at least 100 cc. hydrogen per gram zirconium content. For best results, we use a zirconium content of 0.4 to 0.7% with 125 to 175 cc. hydrogen per 100 g. alloy, a particularly suitable composition being 0.45-0.65% Zr with about 140 cc. hydrogen per 100 gram alloy.

Beryllium may be incorporated in the alloy in amounts up to about 0.01% with a view to improving the oxidation resistance of the alloy (both in the molten state and in the solid state at high temperatures) and also to minimising grain growth during annealing subsequent to working.

We have found that with a full zirconium content, e.g. 0.6-0.7%, it is only possible to dissolve about 0.0015% beryllium in the liquid alloy, the balance of the beryllium content being present in the form of insoluble beryllium rich intermetallic particles. This amount of dissolved beryllium is sufficient to produce detectable reduction in tendency to oxidise, but is far from sufficient to achieve the marked suppression of the burning tendency which can be obtained with beryllium in magnesium and its alloys which do not contain zirconium. We have further found that if the zirconium content of a magnesium-zirconium alloy is decreased, the amount of beryllium which can be taken in solution is increased. Thus, if the zirconium content is reduced to the level of 0.05 to 0.1% the beryllium solubility is raised to about 0.005%, i.e. to

substantially the same level as in pure magnesium. In consequence, such alloys with lowered zirconium content and containing up to 0.005% dissolved beryllium show very advantageous suppression of the tendency to oxidise.

For some purposes, it may be desirable to homogenise the billet or other workpiece before subjecting it to the hydriding step. The zirconium hydride in the final product will then be present in substantially uniform dispersion or diffuse bands, in contrast with material which has been hydrided and extruded without an additional homogenisation; in the latter case the zirconium hydride precipitation is present in narrow, sharply defined bands separated by regions of greater width which are substantially free from zirconium precipitation. Such homogenisation treatment is only worth carrying out where the zirconium content of the alloy exceeds about 0.4%, otherwise the zirconium distribution is more uniform throughout the microstructure and without the relatively small intense concentrations of dissolved zirconium (the well-known "cores") characteristic of alloys with high zirconium content. Alloys prepared by extrusion of homogenised and hydrided billet possess high resistance to grain growth with creep ductility similar to that in the normal extruded state.

According to a further aspect of the invention, therefore, a fine grained wrought zirconium alloy is produced containing at least 0.4% zirconium together with at least 22 cc. hydrogen per 100 g. alloy (with manganese, rare earth metals, thorium, and/or beryllium if desired in the above specified ranges) and with microstructure characterised by the presence of precipitation in substantially uniform dispersion or diffuse bands.

For certain purposes, e.g. fuel element cans operating in the high temperature regions of gas cooled graphite moderated reactors, the reduction in creep ductility associated with the formation of precipitation-free zones in wrought products which have been hydrided after working may not be serious. Accordingly, alloys which have been made by homogenisation followed by extrusion and hydriding treatments may be valuable. The increased stiffness which can be obtained when manufacturing extrusions by this route is also shown in the above table. Low temperature hydride treatment, e.g. 450° C., is desirable to minimise grain growth and surface oxidation on the final product.

According to another aspect of the present invention, therefore, a wrought zirconium alloy exhibiting good resistance to grain growth and good creep resistance at a high temperature contains at least 0.4% zirconium with at least 22 cc. hydrogen per 100 g. alloy, the alloy containing manganese and/or beryllium if desired in the above specified ranges but not rare earth metals and thorium, and a microstructure characterised by the presence of precipitation in substantially uniform dispersion or diffuse bands, together with precipitation-free zones near the grain boundaries.

If desired, a fine grained wrought alloy can be prepared by homogenisation prior to extrusion. In this way, we have made an alloy showing greater stiffness than normal extruded alloys but with equally good creep ductility (see Table I, extrusion G) and good resistance to grain growth. Such a product is not, however, metallurgically stable at high temperatures in moist atmospheres, since it is possible for the zirconium to precipitate as hydride. For the homogenisation treatment the furnace atmosphere should be substantially free from hydrogen or moisture and accordingly the hydrogen content will not exceed 20 cc. per 100 grams of the alloy.

According to a further aspect of the present invention, therefore, a fine grained wrought magnesium alloy with enhanced creep resistance and good grain growth stability contains 0.4 to 0.7% zirconium in substantially uniform solution or in diffuse bands, the alloy containing manganese and/or beryllium if desired as before. The distribution of the zirconium in solution can be readily seen

by subjecting the alloy to a hydriding treatment, e.g. at 500° C. in moist hydrogen, and subsequently etching a polished microsection in 2% nital.

The preferred homogenisation temperature is at least 625° C., and the preferred time at least 24 hrs. Alternatively, a longer period such as 100 hrs. may be used at a lower temperature, e.g. 600° C. It is desirable during homogenisation heat treatments to exclude sources of hydrogen, such as moisture in the atmosphere, until the treatment is complete. Accordingly, heat treatment may be carried out in dry argon, with a fused boric acid coating, or in a sealed container.

We have found that good results can be obtained in accordance with the present invention when starting with either a cast billet or a billet cut from extruded bar.

The excellent resistance to grain growth provided by alloys in accordance with the present invention is illustrated for two of its preferred embodiments in Table II which relates to grain growth after pre-straining 5½% at 250° C., followed by heat treatment for 100 hrs. at 450° C. of an alloy of composition Mg-0.6% Zr.

TABLE II

| Condition                       | Average Grain Size after pre-straining and heat treatment (mm.) |
|---------------------------------|-----------------------------------------------------------------|
| Normal extruded bar             | 0.16                                                            |
| Homogenised, hydrided, extruded | 0.08                                                            |
| Hydrided, extruded              | 0.02                                                            |

Homogenisation treatment: 20 hrs. at 625° C.  
Hydriding treatment: 16 hrs. at 550° C.

The effects achieved with and without the use of this invention are illustrated in the accompanying drawing which diagrammatically shows the microstructure of extruded alloys consisting of 0.5% zirconium, remainder magnesium, at a magnification of 150.

FIGURE 1 shows the alloy which has been hydrided after extrusion.

The structure shows (a) coarse grain, (b) precipitation B in very distinct bands, and (c) precipitation-free zones C alongside the grain boundaries.

The bands of precipitate consist of zirconium hydride and are formed by spreading out of the zirconium-rich solid solution corings when the cast structure is worked. The precipitation-free zones alongside the grain boundaries show that the alloy has been hydrided subsequently to working.

FIGURE 2 shows the alloy when hydrided before extrusion.

The microstructure shows (a) fine grain, (b) precipitation D in very distinct bands and (c) no precipitation-free zones alongside the grain boundaries.

FIGURE 3 shows the alloy when homogenised, then hydrided and finally extruded.

The microstructure shows (a) fine grain, (b) generally uniform precipitation E but with indications of diffuse bands, and (c) no precipitation-free zones near grain boundaries.

Uniformity of the distribution of precipitate shows that the alloy has been homogenised before hydride treatment, and the absence of precipitation-free zones alongside the grain boundaries shows that it has been hydrided before extrusion.

FIGURE 4 shows the alloy when homogenized initially but hydrided after extrusion.

The microstructure shows (a) coarse grain, (b) generally uniform precipitation with indications of diffuse bands, and (c) precipitation-free zones alongside the grain boundaries.

The generally uniform precipitation indicates that the alloy has been homogenized before hydride precipitation, and the precipitation-free zones show that the hydriding treatment was applied after extrusion.

I claim:

1. A wrought magnesium alloy consisting of the following parts by weight:

|       |                                   |
|-------|-----------------------------------|
| Zr    | 0.1-1%.                           |
| H     | At least 22 cc. per 100 g. alloy. |
| Mn    | 0-0.3%.                           |
| R.E.  | 0-3.0%.                           |
| Th    | 0-3.0%.                           |
| 10 Be | 0-0.01%.                          |
| Mg    | Remainder.                        |

the rare earth metals and thorium together not exceeding 4.0%, the hydrogen content being at least 80 cc. per gram zirconium content, and the microstructure of the alloy being characterised in that the distribution of the precipitate does not change in the neighborhood of the grain boundaries.

2. A wrought magnesium alloy as claimed in claim 1, with the following parts by weight:

|    |                              |
|----|------------------------------|
| Zr | 0.1-0.7%.                    |
| H  | 22-350 cc. per 100 g. alloy. |
| Mn | 0-0.2%.                      |
| Mg | Remainder.                   |

the hydrogen content being at least 100 cc. per gram zirconium content.

3. A wrought magnesium alloy as claimed in claim 1 with the following parts by weight:

|    |                              |
|----|------------------------------|
| Zr | 0.25-0.7%.                   |
| H  | 50-250 cc. per 100 g. alloy. |
| Mg | Remainder.                   |

the hydrogen content being at least 100 cc. per gram zirconium content.

4. A wrought magnesium alloy as claimed in claim 1 with the following parts by weight:

|    |                               |
|----|-------------------------------|
| Zr | 0.4-0.7%.                     |
| H  | 125-175 cc. per 100 g. alloy. |
| Mg | Remainder.                    |

5. A wrought magnesium zirconium alloy, having a composition as claimed in claim 1, in which the zirconium content is at least 0.4% and the microstructure is characterised by precipitation in substantially uniform dispersion or in diffuse bands lying in the direction of metal flow.

6. A wrought magnesium zirconium alloy having a composition as claimed in claim 1, excluding rare earth metals and thorium in which the zirconium content is at least 0.4% and the microstructure is characterised by precipitation in substantially uniform dispersion or in diffuse bands lying in the direction of metal flow together with precipitation-free zones near the grain boundaries.

7. A wrought alloy having the following parts by weight:

|    |                                           |
|----|-------------------------------------------|
| Zr | 0.4-0.7%.                                 |
| H  | Not exceeding 20 cc. per 100 g. of alloy. |
| Mn | 0-0.03%.                                  |
| Be | 0-0.01%.                                  |
| Mg | Remainder.                                |

in which the zirconium is present in substantially uniform solution or diffuse bands lying in the direction of metal flow.

8. An alloy as claimed in claim 1, wherein the zirconium content is 0.1-0.4%, beryllium is 0.002-0.005% and manganese is less than 0.2%.

9. A process for producing a wrought magnesium alloy which consists in subjecting a cast or extruded billet or other workpiece of the following parts by weight:

|    |         |       |
|----|---------|-------|
| Zr | percent | 0.1-1 |
|----|---------|-------|

Mn \_\_\_\_\_ do 0-0.3  
 R.E. \_\_\_\_\_ do 0-3.0  
 Th \_\_\_\_\_ do 0-3.0  
 Be \_\_\_\_\_ do 0-0.01  
 Mg \_\_\_\_\_ Remainder

the rare earth metals and thorium together not exceeding 4%, to a hydriding treatment, said hydriding treatment being effected in an atmosphere containing hydrogen in a form capable of being absorbed into the alloy, for at least half an hour at a temperature of at least 300° C., so as to introduce at least 0.002% hydrogen into the alloy and subjecting the workpiece to plastic deformation.

10. A process as claimed in claim 9 in which the billet or other workpiece has the following parts by weight:

Zr \_\_\_\_\_ percent 0.1-0.7  
 Mn \_\_\_\_\_ do 0-0.2  
 Be \_\_\_\_\_ do 0-0.01  
 Mg \_\_\_\_\_ Remainder

11. A process for producing a fine-grained wrought magnesium alloy, which consists in effecting solution heat treatment of a workpiece of magnesium alloy of the following parts by weight:

Zr \_\_\_\_\_ percent 0.4-0.7  
 Mn \_\_\_\_\_ do 0-0.2  
 Be \_\_\_\_\_ do 0-0.01  
 Mg \_\_\_\_\_ Remainder

said heat treatment being effected at a temperature exceeding 575° C. for at least 4 hrs. and subjecting the workpiece to plastic deformation.

12. A process as claimed in claim 9, in which a hydride treatment is carried out at a temperature of 400-600° C. for at least 5 hrs. per in. of maximum section thickness.

13. A process as claimed in claim 9, in which the workpiece is shot-blasted prior to hydride treatment. 35

14. A process as claimed in claim 9, in which the hydride treatment is carried out at a temperature below 500° C.

15. A process as claimed in claim 9, wherein the hydride treatment is effected under a pressure above atmospheric pressure.

16. A process for producing a fine-grained wrought magnesium alloy which consists in effecting solution heat treatment of a workpiece of magnesium alloy of the following parts by weight:

Zr \_\_\_\_\_ percent 0.4-0.7  
 Mn \_\_\_\_\_ do 0-0.2  
 Be \_\_\_\_\_ do 0-0.01  
 Mg \_\_\_\_\_ Remainder

15 said heat treatment being effected at a temperature exceeding 575° C. for at least 4 hrs., subjecting the workpiece to a hydriding treatment in an atmosphere containing hydrogen in a form capable of being absorbed into the alloy at a temperature of at least 300° C. and then subjecting the workpiece to plastic deformation.

References Cited in the file of this patent

UNITED STATES PATENTS

25 2,604,396 Jessup \_\_\_\_\_ July 22, 1952

FOREIGN PATENTS

558,018 Canada \_\_\_\_\_ May 27, 1958

OTHER REFERENCES

30 Ball et al., "Further Progress in the Development of Mg-Zr Alloys to Give Good Creep and Fatigue Properties Between 500° and 650° F." Journal of Metals, trans. AIME, July 1953.